

F. SPARRE.

PROCESS FOR PRODUCING ARTIFICIAL LEATHER.  
APPLICATION FILED SEPT. 3, 1914. RENEWED JULY 10, 1917.

1,257,756.

Patented Feb. 26, 1918.



Witnesses:

Alfred  
J. Newell

Fig. 2.

15 Inventor  
Sir Alfred.  
By Attorney  
Bindle, Wright & Small.

# UNITED STATES PATENT OFFICE.

FIN SPARRE, OF WILMINGTON, DELAWARE, ASSIGNOR TO E. I. DU PONT DE NEMOURS POWDER COMPANY, OF WILMINGTON, DELAWARE, A CORPORATION OF NEW JERSEY.

## PROCESS FOR PRODUCING ARTIFICIAL LEATHER.

1,257,756.

Specification of Letters Patent. Patented Feb. 26, 1918.

Application filed September 3, 1914, Serial No. 859,973. Renewed July 10, 1917. Serial No. 179,768.

To all whom it may concern:

Be it known that I, FIN SPARRE, of Wilmington, in the county of New Castle, and in the State of Delaware, have invented a certain new and useful Improvement in Processes for Producing Artificial Leather, and do hereby declare that the following is a full, clear, and exact description thereof.

My invention relates particularly to an improvement in the methods of producing coated fabrics but more especially woven fabrics bearing a coating or layer of a nitrocellulose composition.

The object of my invention is to produce a product of this kind in which a layer of nitrocellulose composition carried by the fabric will be very effectively and securely anchored to the fabric. It is generally known that fabrics coated with nitrocellulose compositions are sometimes given 14 to 16 coatings, the same being effected by drying and recovery of the solvent after each coating. By this process the anchorage of the coating to the fabric is about all that could be desired. I have conceived the idea of putting on one or more coats in this manner with drying after each coating, just a sufficient number of coatings being applied to obtain good anchorage to the fabric. To obtain the desired final thickness I propose to put a final coating on by means of calender rolls. A cement coat may or may not be applied to the partially coated fabric as it enters the calenders for the application of the final coating.

While my invention is capable of being carried out in many different ways, for purpose of illustration I shall describe only one way in which it may be carried out. The present method of applying jelly coats by means of a doctor blade is well known and it is a combination of this operation with the calender coating with or without intermediate cementing coat that I claim as my invention. For the purpose of illustration I shall show one form of apparatus used in applying the plastic after the fabric has been given one or more jelly coats by the old process.

Figure 1 is a front elevation of a machine which may be used in connection with my process;

Fig. 2 is a side elevation of the same; Fig. 3 is an end elevation in detail of a

shaft on which the fabric is carried when being fed into the machine; 55

Fig. 4 is an end elevation of one of the wooden shuttles used for carrying the fabric;

Fig. 5 is an end elevation of one of the gears; and

Fig. 6 is a plan view of the "doctor" blade 60 provided with ears for feeding the cementing material upon the web of fabric.

In the drawings I have shown a machine having a main frame 1, in which there are carried three rolls 2, 3 and 4. These rolls 2, 3 and 4 are carried upon shafts 5, 6 and 7, respectively. The shaft 6 of the middle roll 3 is maintained in a fixed position in the main frame 1. The shafts 5 and 7, however, are supported in vertically movable boxes 65 8 and 9, which are adapted to be adjusted by means of screws 10 and 11, supported in the main frame 1 and having worm wheels 12 and 13 on their ends which mesh with worms 14 and 15, carried by two shafts 16 70 and 17, and adapted to be operated by handles 18 and 19. The shafts 5, 6 and 7 carry near one end thereof, gears 20, 21 and 22, which are keyed to the shaft by means of removable keys 23, said gears 20, 21 and 22 80 being all of the same size. Upon the other end of the said shafts 5, 6 and 7, are carried gears 24, 25 and 26, the gear 25 being smaller than the gears 24 and 26, and said gears being keyed to their respective shafts in a 85 similar manner to the gears 20, 21 and 22. Only one of these sets of gears is used at a given time. When the gears 20, 21 and 22 are used the keys are removed from gears 24 and 26, and when the gears 24, 25 and 26 90 are used the keys are removed from the gears 20 and 22. The gears 20, 21 and 22 are used when it is desired to have the rolls 2, 3 and 4 moved at the same speed, and the gears 24, 25 and 26 are used when it is desired to have the top and bottom rolls move slower than the middle roll. The central shaft 6 is extended at the one end of the machine so as to carry a large gear 27, which meshes with a small gear 28 having at one 100 end thereof a tight pulley 29 and a loose pulley 30. Guide plates 31 and 32 are supported upon rods 33 and 34 from the main frame 1, said guide plates 31 and 32 fitting against the adjacent faces of the rolls 2 and 105 3 to retain a body of plastic material 35

such as a plastic nitrocellulose composition in place thereon. Near the bottom the main frame 1 supports in a pair of arms 36 a shaft 37 adapted to receive a wooden bobbin 38 carrying a roll of fabric such as cloth to be provided with a coating. A friction band 39 extends around the shaft 37, so as to retard the unwinding of the fabric and therefore maintain it taut. From the shaft 37, the fabric is fed over a guide roll 40, supported in the arms 36, and from this point the fabric passes under a doctor blade 41, supported in arms 42 from the main frame 1, and held in position by thumb screws 43. A body of nitrocellulose jelly or other cementing material 44 is designed to be carried in front of the doctor blade 41, said body of cementing material being confined in its proper position by a pair of angle plates 45, attached by thumb screws 46, to the doctor blade 41.

In carrying out my process I first apply one or more coats of nitrocellulose jelly to the fabric in the usual manner, using a coating or spreading machine of the well-known type. Each of these coats is dried after it is applied. The coated material is then passed to the above described calender machine, where the procedure is as follows:—

30 A coating or cementing material is preferably first applied on top of the coats already applied. This is done by means of the doctor blade 41. Before this cementing coating has dried the goods pass between the rolls 33 and 4 where they receive a coating of plastic material from the body of plastic material 35. Then the coated fabric may be conveyed away and supported in such a manner as to permit the coatings to dry and harden.

In the application of plastic coatings to fabrics by means of calender rolls the greatest difficulty hitherto experienced has been in obtaining an efficient anchorage of the coating to the fabric. My invention involves the above described novel method of obtaining this anchorage by first applying to the fabric one or more coats in a spreading machine and then applying the main body 50 of the coating by a calender machine on top of these preliminary coats. The intermediate cementing coat is not essential but will usually be found to be advantageous. My invention may be carried out with many 55 different coating compositions, and the particular type of spreading machine used for applying and drying the preliminary anchorage coats is not material.

While I have described my invention 60 above in detail, I wish it to be understood

that many changes may be made therein without departing from the spirit of my invention.

I claim:

1. The process of producing a coated fabric, which comprises applying to the fabric one or more coats of a film-producing nitrocellulose composition, each coat being dried after its application, and then applying a coating of plastic material in sheet form by means of pressure. 65

2. The process of producing a coated fabric, which comprises applying to the fabric one or more coats of film producing nitrocellulose composition, each coat being dried 75 after its application, and then applying a coating of nitrocellulose plastic by means of pressure.

3. The process of producing a coated fabric, which comprises applying to the fabric 80 one or more coats of nitrocellulose composition in the form of a jelly, each coat being dried after its application, then applying a coating of cementing material, and then before the cementing material has been al- 85 lowed to dry applying a coating of nitrocellulose plastic by means of pressure.

4. The process of producing a coated fabric, which comprises applying to the fabric one or more coats of a film-producing nitro- 90 cellulose composition, each coat being dried after its application, and then applying a coating of plastic cellulose composition by means of calender rolls.

5. The process of producing a coated fab- 95 ric, which comprises applying to the fabric one or more coats of nitrocellulose composition in the form of a jelly, each coat being dried after its application, then applying a coating of cementing material, and then 100 before the cementing material has been allowed to dry applying a coating of nitrocellulose plastic by means of calender rolls.

6. The process of producing a coated fab- 105 ric, which comprises applying to the fabric one or more coats of nitrocellulose composition in the form of a jelly, each coat being dried after its application, then applying a coating of nitrocellulose cementing ma- 110 terial, and then before the cementing ma- terial has been allowed to dry applying a coating of nitrocellulose plastic by means of pressure.

In testimony that I claim the foregoing I have hereunto set my hand.

FIN SPARRE.

Witnesses:

HAMILTON BRADSHAW,  
JAMES H. LEACH.